

## UNITED STATES PATENT OFFICE

2,149,253

METHOD OF TREATING METAL SURFACES  
TO INHIBIT CORROSION

Harry A. Cooper, Maplewood, N. J.

No Drawing. Application May 19, 1937,  
Serial No. 143,531

1 Claim. (Cl. 29—90)

This invention relates to metal coating processes and more particularly to a method of coating articles made of corrodible metals such as iron or steel with a thin coating of stainless steel or other corrosion-resisting metals or alloys of metals.

An object of this invention is to provide during the process of cleaning and polishing a method of rendering corrosion-resistant objects made of corrodible metals such as iron and steel.

A further object is to provide a method of cleaning and polishing objects made of stainless steel or other corrosion-resisting metals or alloys of metals to give them a lasting and durable finish and a non-corrodible surface.

The outstanding disadvantage in the use of iron and steel for manufacturing purposes is the rapid corrosion of the surfaces exposed to oxidation. There are many expedients employed to overcome this disadvantage i. e. galvanizing, cadmium plating, nickel plating, painting, etc. These expedients necessitate extra steps and special processes and equipment after the article is otherwise complete and add materially to the time and cost of manufacture. I have discovered a method of rendering objects made of corrodible metals such as iron and steel corrosion-resistant during the process of cleaning and polishing without adding to the cost of the finished article.

Heretofore the use of steel balls or shot in cleaning and polishing objects made of stainless steel and other alloys has resulted in a tendency for the object to corrode easily. I have discovered that in the process of cleaning and polishing, the steel balls or shot deposit a thin coating of ordinary steel on the object, thus destroying the most valuable property of the stainless steel or alloy. By using the method hereinafter described this tendency toward corrosion disappears and the object retains all the desirable properties inherent in stainless steel or the particular metal or alloy used.

The process consists of bringing pellets such as shot, punchings, filings or the like, made of stainless steel or other corrosion-resisting metals or alloys of metals into forcible contact with the object which is being cleaned and coated. This is accomplished in the conventional manner either by forcing the pellets against the object by compressed air or mechanical means or by tumbling the object in the presence of the pellets.

In all cases of corrodible metals or alloys the coating pellets should be of a softer metal than the object being coated, so that as the softer pellets forcibly hit the object, a minute quantity of the stainless steel or corrosion-resisting metals or alloys of metals is deposited on the surface of the object. As the process is continued the object will become covered with a thin, closely adhering pellicle or coating of stainless steel or the corrosion-resisting metals or alloys of metals. In the case of objects made of stainless steel or corrosion-resisting metals or alloys of metals, pellets of a similar metal or alloy should be used.

The use of pellets made of stainless steel or other corrosion-resisting metals or alloys of metals in the cleaning and polishing of objects made of corrodible metals such as iron or steel, results in the deposit of a corrosion-resisting coating on the surface of the object. It has been found that when corrosion-resisting pellets are substituted for the ordinary steel pellets in the process of cleaning and polishing objects made of stainless steel or other corrosion-resisting metals or alloys of metals, there results a product with much higher corrosion-resisting qualities.

What I claim is:

The method of cleaning and polishing stainless steel objects which consists in forcibly contacting the surface of the object with stainless steel pellets.

HARRY A. COOPER. 40